

# United States Patent Office

3,508,911

Patented Apr. 28, 1970

1

3,508,911

## LOW CARBON STEEL WITH TITANIUM ALUMINUM AND BORON

John Y. Riedel, Bethlehem, Pa., assignor to Bethlehem Steel Corporation, a corporation of Delaware  
No Drawing. Filed May 11, 1967, Ser. No. 637,617  
Int. Cl. C22c 39/02

U.S. Cl. 75—124

7 Claims

### ABSTRACT OF THE DISCLOSURE

A hypoeutectoid boron steel containing small amounts of aluminum, titanium and, optionally, columbium, which is readily weldable and which can be heat treated to provide a combination of high yield strength and low V-Notch Charpy impact transition temperature and in heavier sections than prior art steels.

### BACKGROUND OF THE INVENTION

This invention pertains to the composition of a novel hypoeutectoid boron steel containing aluminum and titanium and, optionally, columbium and which has been heat treated to provide a microstructure which is predominately tempered martensite.

It is well known that as much as several percent of the elements from the group consisting of manganese, silicon, nickel, chromium and molybdenum have a bene-

5 known hardenability improving constituents from the group consisting of manganese, silicon, nickel, and molybdenum and will fall within the limits shown on Table I. The alloys of this invention do not contain significant amounts of either chromium or vanadium.

TABLE I

|    |                              | Broad      | Narrow    |
|----|------------------------------|------------|-----------|
| 10 | Carbon.....                  | .10/.30    | .12/.21   |
|    | Manganese.....               | .20/1.00   | .45/.75   |
|    | Phosphorous.....             | 1.05       | 1.00      |
|    | Sulphur.....                 | 1.05       | 1.05      |
| 15 | Silicon.....                 | .10/.75    | .20/.35   |
|    | Nickel.....                  | 13.00      | 13.00     |
|    | Chromium.....                | 1.20       | 1.20      |
|    | Molybdenum.....              | 13.00      | 13.00     |
|    | Aluminum.....                | .02/.20    | .05/.10   |
|    | Titanium.....                | .01/.04    | .01/.03   |
|    | Columbium <sup>2</sup> ..... | .01/.13    | .02/.05   |
|    | Boron.....                   | .0005/.005 | .001/.005 |
|    | Vanadium.....                | 1.05       | 1.05      |

<sup>1</sup> Maximum. <sup>2</sup> Optional.

20 The balance being essentially iron. All compositions are shown as percentages based on weight.

Table II shows a summary of the yield strength and V15 transverse Charpy transition temperature determinations made on specimens of various thicknesses of plate steel having compositions within the broad ranges of 25 compositions of Table I. All of the steel plates were heat treated by water quenching from 1650° F. and tempering at 1200° F. so as to provide a microstructure which was predominately tempered martensite.

TABLE II

| Specimen No. | Thickness<br>(in.) | C   | Mn  | Si  | Ni    | Mo  | Al   | Ti   | Cb    | B    | Yield<br>strength,<br>p.s.i. | Transition<br>temp.,<br>°F. |
|--------------|--------------------|-----|-----|-----|-------|-----|------|------|-------|------|------------------------------|-----------------------------|
| 1.....       | 3/4                | .18 | .55 | .29 | ..... | .55 | .07  | .02  | ..... | .003 | 107,000                      | -75                         |
| 2.....       | 3/4                | .20 | .58 | .25 | ..... | .55 | .09  | .02  | ..... | .003 | 109,000                      | -125                        |
| 3.....       | 3/4                | .18 | .59 | .32 | ..... | .55 | .08  | .03  | ..... | .004 | 117,000                      | -110                        |
| 4.....       | 3/4                | .16 | .82 | .34 | ..... | .52 | .10  | .017 | ..... | .002 | 112,700                      | -120                        |
| 5.....       | 3/4                | .16 | .82 | .34 | ..... | .52 | .10  | .017 | ..... | .002 | 113,000                      | -155                        |
| 6.....       | 3/4                | .16 | .82 | .34 | ..... | .52 | .10  | .017 | ..... | .002 | 110,400                      | -95                         |
| 7.....       | 3/4                | .16 | .82 | .34 | ..... | .52 | .10  | .017 | ..... | .002 | 106,300                      | -85                         |
| 8.....       | 3/4                | .19 | .68 | .25 | .02   | .57 | .07  | .02  | ..... | .002 | 116,350                      | -70                         |
| 9.....       | 3/4                | .18 | .55 | .30 | ..... | .55 | .08  | .02  | ..... | .003 | 122,000                      | -12.5                       |
| 10.....      | 3/4                | .18 | .55 | .31 | ..... | .53 | .07  | .01  | ..... | .003 | 113,700                      | -50                         |
| 11.....      | 3/4                | .18 | .60 | .37 | ..... | .54 | .06  | .01  | ..... | .004 | 115,000                      | -110                        |
| 12.....      | 1                  | .19 | .67 | .26 | 1.36  | .64 | .068 | .026 | ..... | .003 | 135,800                      | -110                        |
| 13.....      | 2                  | .19 | .67 | .26 | 1.36  | .64 | .068 | .026 | ..... | .003 | 109,000                      | -150                        |
| 14.....      | 2 1/2              | .19 | .67 | .26 | 1.36  | .64 | .068 | .026 | ..... | .003 | 101,700                      | -150                        |
| 15.....      | 2                  | .20 | .67 | .34 | 1.51  | .66 | .07  | .026 | ..... | .006 | 106,300                      | -150                        |

ficial effect on the hardenability of hypoeutectoid boron steels. It is also known that when these steels have a microstructure which is predominately tempered martensite they will provide a minimum yield strength of approximately 90,000 p.s.i. in sections up to approximately 1" in thickness.

50 Specimens 1-7 illustrate the properties obtained with the heat treated hypoeutectoid aluminum-titanium-boron steels of this invention. Specimens 8-15 illustrate the properties obtained with the heat treated hypoeutectoid aluminum-titanium-columbium-boron steels of this invention.

### DESCRIPTION OF THE PREFERRED EMBODIMENT

55 It has now been discovered that the addition of small amounts of aluminum and titanium to hypoeutectoid boron steel improves the yield strength and V15 Charpy transition temperature when the microstructure is predominately tempered martensite. These aluminum and titanium additions do not affect the as-quenched hardenability as measured by an end quench test, but the improved properties of the steel of this invention are apparent in heavier sections, e.g. 1 1/4" thick over similar steels which do not contain aluminum and titanium. It has also been discovered that the addition of a small amount of columbium to the above hypoeutectoid aluminum, titanium, boron steel will provide either an additional increase in yield strength without adversely affecting the V15 Charpy transition temperature or an equivalent yield strength and transition temperature in even greater thicknesses, e.g. 2 1/2" thick.

The hypoeutectoid steel of this invention may contain as much as several percent of one or more of the well

55 The steel compositions of this invention are preferably made by adding silicon, aluminum, titanium (columbium is optional), and boron, in that sequence, to a ladle into which a partially deoxidized hypoeutectoid steel melt is being poured as is described in my copending application Ser. No. 626,430 filed Mar. 28, 1967.

60 A specific example of producing the novel hypoeutectoid boron steel of this invention is as follows:

65 1. A basic open hearth steel melt of the following composition was produced in the usual manner.

|          |      |          |      |
|----------|------|----------|------|
| C .....  | .12  | Si ..... | .002 |
| Mn ..... | .13  | Ni ..... | .02  |
| P .....  | .012 | Cr ..... | .04  |
| S .....  | .032 | Mo ..... | .56  |

70 2. The melt was blocked by adding spiegeleisen and silicomanganese to the metal in the furnace.

3. The heat was tapped from the furnace at a temperature of 2890° F. into a ladle containing sufficient 50% ferrosilicon to recover approximately .25% silicon.

4. As the heat was being tapped into the ladle additions of carbon (coke), aluminum, titanium and ferroboron (13% boron) were made to the ladle in that sequence.

5. The ladle analysis was as follows:

|    |      |    |      |    |
|----|------|----|------|----|
| C  | .19  | Cr | .05  |    |
| Mn | .68  | Mo | .57  | 10 |
| P  | .010 | Al | .08  |    |
| S  | .021 | Ti | .025 |    |
| Si | .25  | B  | .002 |    |
| Ni | .02  |    |      |    |

The ladle was teemed into ingot molds equipped with hot tops. The ingots were stripped five hours after being poured and heated to 2440-2460° F. for rolling into slabs. The slabs were reheated to 2350-2400° F. and rolled into plates. Finishing temperatures varied between 1870 and 1480° F. Sample No. 8 on Table II shows the composition and properties of a sample heat treated plate from this heat.

In another specific example a 190 ton heat of steel was produced in the same manner as the previous example except that the base steel contained approximately 1.35% nickel and ferrocolumbium was added to the ladle after the titanium addition and before the ferroboron addition. Specimens 12-15 of Table II illustrate the composition and properties of sample heat treated plates made from this steel.

The novel steel compositions of this invention can be heat treated to a microstructure which is predominately tempered martensite in sections up to at least 2½" thick so as to provide a weldable steel having minimum yield strength of 100,000 p.s.i. in combination with a V15 Charpy transition temperature not higher than -50° F. in a direction transverse to the major direction of rolling.

In the specific examples the details of methods and the compositions are only intended as illustrations of this invention which is defined in the following claims.

1. A steel consisting of:

|           |            |         |
|-----------|------------|---------|
| Carbon    | .10/.30    | Percent |
| Manganese | .20/1.00   |         |
| Silicon   | .10/.75    |         |
| Aluminum  | .02/.20    |         |
| Titanium  | .01/.04    |         |
| Boron     | .0005/.005 |         |

the balance being essentially iron.

2. The steel of claim 1 which also contains .01/.13% columbium.

3. A hypoeutectoid steel having a microstructure which is predominately tempered martensite and consisting of:

|           |           |            |         |
|-----------|-----------|------------|---------|
| Carbon    | (minimum) | .10        | Percent |
| Manganese |           | .20/1.00   |         |
| Silicon   |           | .10/.75    |         |
| Aluminum  |           | .02/.20    |         |
| Titanium  |           | .01/.04    |         |
| Boron     |           | .0005/.005 |         |

balance essentially iron.

4. The steel of claim 3 which also contains .01/.13% columbium.

5. A steel article having a microstructure which is predominately tempered martensite characterized by a yield strength of at least 100,000 p.s.i. in combination with a V15 transverse Charpy transition temperature not higher than -50° F., the said steel consisting of:

|            |           |           |
|------------|-----------|-----------|
| Carbon     | .12/.21   | Percent   |
| Manganese  | .45/.70   |           |
| Phosphorus | (maximum) | .035      |
| Sulphur    | do        | .040      |
| Silicon    |           | .20/.35   |
| Nickel     | (maximum) | 3.00      |
| Chromium   | do        | .20       |
| Molybdenum | do        | 3.00      |
| Aluminum   |           | .05/.10   |
| Titanium   |           | .01/.03   |
| Vanadium   | (maximum) | .05       |
| Boron      |           | .001/.005 |

the balance being essentially iron.

25 6. The steel of claim 5 which also contains .02/.05% columbium.

7. A steel article having a microstructure which is predominately tempered martensite characterized by a yield strength of at least 110,000 p.s.i. in combination with a V15 transverse Charpy transition temperature not higher than -50° F. in sections up to 2½" in thickness, said steel consisting of:

|            |           |           |
|------------|-----------|-----------|
| Carbon     | .12/.21   | Percent   |
| Manganese  | .45/.70   |           |
| Silicon    | .20/.35   |           |
| Nickel     | (maximum) | 3.00      |
| Chromium   | do        | .20       |
| Molybdenum | do        | 3.00      |
| Aluminum   |           | .05/.10   |
| Titanium   |           | .01/.03   |
| Vanadium   | (maximum) | .05       |
| Columbium  |           | .02/.05   |
| Boron      |           | .001/.005 |

the balance being essentially iron.

50 7. References Cited  
UNITED STATES PATENTS

|           |         |          |        |
|-----------|---------|----------|--------|
| 2,853,379 | 9/1958  | Althouse | 75-124 |
| 2,858,206 | 10/1958 | Boyce    | 75-126 |
| 3,198,630 | 8/1965  | Tarwater | 75-124 |
| 3,288,600 | 11/1966 | Johnser  | 75-126 |
| 3,418,110 | 12/1968 | Goda     | 75-124 |

HYLAND BIZOT, Primary Examiner

UNITED STATES PATENT OFFICE  
CERTIFICATE OF CORRECTION

Patent No. 3,508,911 Dated April 28, 1970

Inventor(s) John Y. Riedel

It is certified that error appears in the above-identified patent and that said Letters Patent are hereby corrected as shown below:

Column 2, Table I, line 10, under the column "Narrow" "phosphorous" should read -- .05 maximum -- and not ".00 maximum".

Signed and sealed this 1st day of September 1970.

(SEAL)  
ATTEST:

EDWARD M. FLETCHER, JR.  
Attesting Officer

WILLIAM E. SCHUYLER, JR.  
Commissioner of Patents

### Disclaimer

3,508,911.—*John Y. Riedel*, Bethlehem, Pa. LOW CARBON STEEL WITH TITANIUM ALUMINUM AND BORON. Patent dated Apr. 28, 1970. Disclaimer filed Aug. 24, 1971, by the assignee, *Bethlehem Steel Corporation*.

Hereby disclaims the portion of the term of the patent subsequent to Apr. 20, 1987.

[*Official Gazette October 19, 1971.*]

UNITED STATES PATENT OFFICE  
CERTIFICATE OF CORRECTION

Patent No. 3,508,911 Dated April 28, 1970

Inventor(s) John Y. Riedel

It is certified that error appears in the above-identified patent and that said Letters Patent are hereby corrected as shown below:

The Disclaimer attached to the printed copies, was erroneously printed and should be canceled.

Signed and Sealed this  
*twenty-seventh* Day of *April 1976*

[SEAL]

Attest:

**RUTH C. MASON**  
*Attesting Officer*

**C. MARSHALL DANN**  
*Commissioner of Patents and Trademarks*